

Sept. 26, 1939.

B. M. CARTER

2,174,185

PROCESS FOR ROASTING ORE

Filed March 16, 1938

2 Sheets-Sheet 1



INVENTOR  
Bernard M. Carter  
BY Joseph A. Ryan  
ATTORNEY

Sept. 26, 1939.

B. M. CARTER

2,174,185

PROCESS FOR ROASTING ORE

Filed March 16, 1938

2 Sheets-Sheet 2



INVENTOR  
Bernard M. Carter  
BY Joseph G. Rymer  
ATTORNEY

## UNITED STATES PATENT OFFICE

2,174,185

## PROCESS FOR ROASTING ORE

Bernard M. Carter, Montclair, N. J., assignor to  
 General Chemical Company, New York, N. Y.,  
 a corporation of New York

Application March 16, 1938, Serial No. 196,201

17 Claims. (Cl. 75-9)

This invention relates to roasting of metal sulfide fines by suspension methods of the type disclosed in Cordy and Burgoyne United States Patent 1,758,188 of May 13, 1930.

- 5       Oxidation of metal sulfide, iron pyrites for example, is an exothermic reaction liberating large quantities of heat. In a situation where a commercial suspension roaster of given size is operated to produce, at the burner exit, say a 10% 5  
 10      SO<sub>2</sub> gas, there is a maximum pyrites tonnage which may be satisfactorily desulfurized in a day. With normal radiation from the furnace shell, the heat evolved by combustion of the pyrites with production of a 10% SO<sub>2</sub> gas is distributed, in a representative operation, approximately as follows: the gaseous products of combustion 70-80%; radiation loss 10-20%; cinder 10%. In commercial operation, the gas temperature prevailing in suspension burners ranges 10  
 15      from about 1800° F. to about 1900° F. and is generally around 1850° F. The gas temperatures in the burner should not be permitted to rise appreciably above a maximum of say 1900° F., especially in the zone in which cinder collects just 15  
 20      prior to discharge from the furnace, because the iron oxide cinder would cease to be free-flowing and would become soft and sticky, thus preventing normal discharge of cinder from the furnace and otherwise interfering with operation 20  
 25      30 to the extent of rendering the same impracticable. In a given burner, the total amount of heat generated is directly proportional to the amount of pyrites burned, heat loss by cinder is relatively small and is directly proportional 30  
 35      35 to the ore charge, and heat loss by radiation is constant. Since gas temperatures should not exceed a maximum, it will be seen a given furnace has a maximum pyrites capacity. For example, it may be assumed that in production 35  
 40      40 of a 10% SO<sub>2</sub> gas, the maximum daily pyrites capacity of such given furnace is 50 tons.
- It would be highly desirable to operate such a burner so as to produce a stronger say 12% SO<sub>2</sub> gas to permit utilization of a smaller wet purification and converter units of the succeeding H<sub>2</sub>SO<sub>4</sub> plant. However, since in production of strong SO<sub>2</sub> gas, avoidance of excessive temperatures may be had only by cutting down the 45  
 45      50 amount of sulfide ore burned, in order to produce the stronger 12% SO<sub>2</sub> gas and yet prevent burner exit gas temperatures in excess of permissible maximum, it would be necessary to reduce the sulfide ore charge to roughly 30 tons.
- 55      One of the objects of the present invention is
- to provide a method by which a given burner of the type disclosed in the Cordy patent may be operated so as to produce the strong SO<sub>2</sub> gas desired without (as hereafter explained) having to reduce, for example by about 40%, the amount of sulfur fed into the burner. The invention aims to provide a sulfide ore roasting process by which all plant units may be substantially reduced in size, or alternatively by which the H<sub>2</sub>SO<sub>4</sub> production of all existing plant units succeeding a given burner may be largely increased. Another object of the invention is to accomplish the desired results by use, in conjunction with the roasting of the metal sulfide fines, of iron sulfate which is of little if any market value and which for all practical purposes may be considered a waste product. A further object of the invention is to provide a method for the economic recovery of the sulfur and iron values contained in iron sulfate. 20
- Certain industrial operations, for example pickling of steel and manufacture of titanium pigments, result in production of large quantities of waste or spent liquors containing as their chief ingredients free sulfuric acid and iron sulfate largely in the ferrous condition. Disposal of these waste liquors presents serious problems to the industries involved. Objections to prior processes for recovery of H<sub>2</sub>SO<sub>4</sub> and FeSO<sub>4</sub> are such that the value of the recovered acid in some instances will be insufficient to cover the operating costs and will in no case yield a return on investment since no economic method of recovering values of iron sulfate is available, and there is no tonnage outlet for iron sulfate either in the form of the monohydrate, FeSO<sub>4</sub>.H<sub>2</sub>O, or the heptahydrate FeSO<sub>4</sub>.7H<sub>2</sub>O. 25
- Another object of the invention is to provide such a method for the recovery of iron and sulfur from iron sulfate that it becomes possible to dispose of waste H<sub>2</sub>SO<sub>4</sub>-FeSO<sub>4</sub> liquors in such a way as to not only cover disposal and operating costs but also to provide a return on the disposal plant investment. 30
- Although the process of the invention is readily adaptable to use of several other substances as initial raw materials, speaking with respect to the preferred embodiment in which iron sulfide and iron sulfate are employed, I have found that by introducing iron sulfide fines, iron sulfate fines, and oxygen into a suspension roaster combustion zone heated to temperatures above the ignition point of the iron sulfide fines, and by regulating the amounts of iron sulfide fines, iron sulfate fines and oxygen introduced so that the 35

roasting operation is effected in such a way as to maintain in the combustion zone temperatures about or above dissociation temperature of sulfur trioxide but preferably not above temperatures which would cause iron oxide cinder at the point of discharge from the roaster to fuse and set up as a solid cake, the iron sulfide fines are roasted to produce iron oxide cinder and sulfur dioxide gas; the iron sulfate is decomposed to form iron oxide cinder, sulfur dioxide and sulfur trioxide gases; the sulfur trioxide formed by decomposition of the iron sulfate is dissociated to sulfur dioxide and oxygen; and the sulfur and iron values of the iron sulfide and of the iron sulfate are recovered as a concentrated sulfur dioxide gas and as relatively free-flowing iron oxide cinder.

I have found that by so proceeding, with respect to a given burner, the iron sulfide input limitation previously mentioned is eliminated and the iron sulfide capacity is materially increased; limitation as to  $SO_3$  concentration is eliminated; the actual and potential heat in a burner, that is actual and potential heat, over and above that needed to keep the burner at operating temperatures is absorbed by and used to decompose iron sulfate. Further, decomposition of iron sulfate to iron oxide and  $SO_2$  is effected without consumption of carbonaceous reducing agent and without taking any special steps, other than those usually involved in suspension roasting of sulfide fines, to create in the combustion zone temperatures high enough to dissociate  $SO_3$  to  $SO_2$  and oxygen. Iron sulfate is decomposed to form the usually sought for suspension roasting products, iron oxide and  $SO_2$ , without incurring expense of independent operations necessitating apparatus, fuel, and operating charges. By reason of the facility with which a concentrated  $SO_2$  gas may be produced, hereinafter explained material reduction in size may be obtained in each plant unit, namely, the burner, the purification system, the drying unit, the converter system, and the absorption system. Furthermore, I am enabled to secure all of these and further advantages which will appear as the description proceeds by utilizing in conjunction with the suspension roasting of iron sulfides a material, iron sulfate, for which there is no appreciable market outlet and for which reason economic recovery of iron and sulfur values from waste industrial  $H_2SO_4$ — $FeSO_4$  liquors has not been possible previously.

Fig. 1 of the drawings illustrates partly in section and partly diagrammatically a plant layout in which a preferred embodiment of the invention may be carried out; and Fig. 2 similarly represents apparatus in which a modified process may be practiced.

Referring to Fig. 1, shaft furnace 10 comprises a vertically elongated preferably cylindrical steel shell 11. Since on account of the nature of the invention it is now possible to use in the roasting operation all of the heat which can be generated by combustion of sulfides, radiation of heat from the burner shell need no longer be relied upon to provide for dissipation of some excess heat. Accordingly, the burner is preferably well insulated to cut down radiation heat loss as far as feasible, and for this reason a layer 14 of insulating material such as Silocel may be interposed between shell 11 and the customary firebrick lining 15.

A mixture of finely divided sulfide ore and finely divided iron sulfate suspended in air or

other oxidizing gas is fed into the upper end of roasting chamber 17 by feed mechanism 18 shown diagrammatically on the drawings. The feed device may include an upwardly projecting cylindrical casing 20 having the lower end set into the crown of the furnace and the upper end closed off by plate 21 provided with a circular opening to accommodate a sulfide-sulfate mixture inlet conduit 23. The diameter of conduit 23 is considerably less than that of casing 20 so as to form an annular air chamber 25 between the outer surface of the conduit and the inner surface of casing 20. A mixture of finely divided sulfide ore and iron sulfate may be continuously fed into conduit 23 by a screw conveyor 26 associated with hopper 27.

Air, serving to effect the suspension of sulfide and iron sulfate fines and to support combustion of sulfides in the roasting chamber, is introduced into the feed mechanism through the inlet 30. The conduit 23 may be provided with a series of openings 31 to permit admission of air from the annular chamber 25 into the interior of conduit 23 to bring about suspension of sulfide fines and iron sulfate fines in air. The particular feed mechanism illustrated constitutes no part of the present invention. Accordingly, any desirable means for forming a suspension of sulfide and iron sulfate fines in oxidizing gas and introducing such suspension into the upper end of the roasting chamber 17 may be employed. For example, mechanism adapted for this purpose is fully described in the Cordy patent.

The bottom of the roasting chamber is funnel-shaped and is provided with a suitable device 32 for removing cinder from the furnace at any desired rate. The  $SO_2$  gas outlet 33 communicates through conduit 34 with the bottom of a supplemental combustion and dust settling chamber 35 provided at the bottom with a dust discharge air lock 36. The top of chamber 35 is connected by flue 37 with inlet header chamber 38 of heat exchanger 40, the inwardly sloping lower portion of the walls of which terminates in an air-lock 41 arranged to permit removal of dust without admission of air. Transferrer 40 may be of any approved construction, although in the embodiment illustrated, is the fire-tube type, an incoming air heating chamber being formed by the exterior of tubes 43, the upper and lower tube sheets, and the intermediate inner surface of the walls of the shell. Since the  $SO_2$  gases introduced into the top of transferrer 40 are highly destructive at the prevailing high temperatures, caution should be taken to construct all metal parts in contact with the gases of sufficiently resistant material such as chrome steel. The gas outlet header chamber 45 is connected through gas conduit 46 with inlet header chamber 48 of a second heat exchanger 50 provided at the bottom with a dust discharge air-lock 51. Design of exchanger 50 is the same as that of 40. The reason for using two exchangers is that since  $SO_2$  gases entering the bottom of exchanger 50 are considerably cooler than the burner exit gases, the tube section of exchanger 50 may be made of ordinary grade of steel. Exchangers 40 and 50 are preferably arranged with tubes 43 and 56 vertical so that dust separating from the  $SO_2$  gases may drop into the lower ends of the transferrers and not clog up the tubes.

Air is pumped by blower 53 through conduit 54 into the space surrounding tubes 56 in exchanger 50, through conduit 58 into the space surrounding tubes 43 in transferrer 40 and then through line 60 to feed mechanism air inlet 30.

5 Gas outlet header chamber 62 of transfer 50 is connected through conduit 63 with a cyclone dust separator 65 which may be comparatively small in size and made of ordinary sheet iron or steel. Gases from which major portion of the dust has been removed by separator 65 pass through line 66 to a wet purification plant 67 which may be of the type disclosed in the Herreshoff Patents 940,595 of November 16, 1909, and 10 1,113,437 of October 13, 1914. Drying system 68, blower 68', contact unit 69 and the absorption system 70 may be of standard design.

10 In the apparatus of Fig. 2, shaft furnace 72, dust collector 73, wet purification plant 74, drying system 75, contact unit 76, and absorption system 77 are the same as in Fig. 1. However, in the operation of the process as carried out in the apparatus of Fig. 2 the air consumed in combustion chamber 78 of furnace 72 is fed into the 15 system by a blower 80, passed through a standard drying tower 81, and introduced through line 82 into air inlet 30 of feed mechanism 18. Gas outlet 84 of furnace 72 communicates through conduit 85 with the bottom of a supplemental combustion and dust chamber 87 provided at the bottom with a dust discharge air-lock 88. The top of chamber 87 is connected by pipe 90 with the inlet header chamber 92 of a waste heat boiler 94, the lower portion of the 20 walls of which terminates in an air-lock 95 arranged so as to permit discharge of dust without admission of air. Boiler 94 may be of any approved construction, and in the embodiment illustrated is of the fire-tube type, the water and 25 steam chamber being formed by the exterior of tubes 96, the upper and lower tube sheets, and the intermediate inner surface of the shell walls. Water may be fed in the space surrounding the tubes through an inlet 98, and steam or hot water 30 withdrawn through outlet 99. A suitable pressure regulator is indicated at 100. Gas outlet header chamber 102 is connected through conduit 104 with a cyclone dust separator 73.

35 An understanding of the nature of the invention and of its many operating advantages may be had by initially considering, as a basis for comparison, what may be deemed a representative example of prior operation of a pyrites suspension burner and the associated  $H_2SO_4$  plant. Such plant comprises five principal units: 40 suspension burner; wet purification system, drying unit; converter unit; and an  $SO_3$  absorption system. As a starting point, it may be assumed that the gas purification system is in accordance with 45 conventional practice and initially designed to handle a gas, say of 10%  $SO_2$  concentration. Hence, by regulation of the amounts of sulfide fines and air introduced, the burner is operated so as to produce a gas containing about 10%  $SO_2$  and 8% oxygen. In this situation, the wet 50 purification exit gas would likewise contain about 10%  $SO_2$  and about 8% oxygen. While theoretically one volume of  $SO_2$  reacts with 0.5 volume of  $O_2$  to form  $SO_3$  in the converters, in practice 55 in order to obtain commercial conversion the amount of oxygen needed should be in excess of the theoretical requirement, and for practical purposes the gas fed to the converter should contain  $SO_2$  and  $O_2$  in ratio of about 1:1.1. Thus, in the case of a 10%  $SO_2$  pyrites gas, more air should be fed into the gas stream to provide the requisite oxygen in the converter. This may be accomplished by introducing the additional air needed just ahead of the drying system, as through an air inlet 133, Fig. 1 of the drawings. In the case 60

65 of a 10%  $SO_2$  pyrites burner gas, the extra air needed dilutes the gas stream to an  $SO_2$  concentration of about 8.5%. Accordingly, where the purification system is initially designed for a 10%  $SO_2$  gas, the converter unit would be designed to handle an 8.5%  $SO_2$  gas.

70 Example 1 of Table I appended to this specification summarizes operation of such a plant. The burner used (Item 2) is a given standard, for instance as shown in the Cordy patent. The 10 purification system (Item 11) is designed for a 10%  $SO_2$  pyrites gas, and the drying, converter and absorption systems (Item 15), for reasons just indicated, are designed to handle an 8.5%  $SO_2$  gas. For reasons explained in the second 15 paragraph of this specification, in the production of a gas of given  $SO_2$  concentration a given furnace has a definite maximum pyrites capacity. It may be assumed that in the production of a 10%  $SO_2$  gas the maximum daily pyrites capacity 20 of such given furnace is 50 tons (Example 1, Item 3) and on this basis it may be considered that the burner is operated at 100% (sulfur output) capacity. The temperature of the burner exit gas is 1850° F. (Item 9).

25 On account of high construction and maintenance costs of the purification system, it would be highly desirable to operate the burner to form a stronger gas, say 12%  $SO_2$  to permit utilization of smaller purification units. The given burner is readily adaptable to produce a stronger gas. 30 However, it will be understood that in formation of a 12%  $SO_2$  gas, the amount of air introduced into the furnace is necessarily reduced, and the temperature of the gas in roasting zone tends to rise correspondingly. The only way to avoid excessive temperatures in the combustion zone is by reducing the tonnage of ore fed into the roaster. For example, commercial practice has shown that where a given burner had a daily 35 pyrites capacity of about 50 tons on production of a 10%  $SO_2$  gas, when the same burner was operated with the same ore and at the same burner temperature so as to supply a 12%  $SO_2$  gas, it was necessary to cut down the ore feed 40 to the burner to about 30 tons. Such an operation is summarized in Example 2 of Table I which shows that to supply the stronger gas to 45 purification, the burner can be operated at only 58% capacity with the result that the  $H_2SO_4$  50 output of the plant as a whole is only 58% of the normal output of Example 1.

55 If an operator wishes to feed to purification a 12% gas for the purpose of effecting economies resulting from the use of a smaller purification unit and at the same time maintain his normal  $H_2SO_4$  production he has available as one alternative installation of an additional or supplementary burner about 70% as large as the initial given burner. Operation of this alternative is 60 summarized in Example 3, the plant of which requires construction and use of a supplemental burner, which partially offsets advantages normally resulting from the 17% smaller purification unit.

65 The second alternative available to the operator is to increase the size of the initial burner. However, this alternative involves difficulties. Normal burner radiation loss decreases as the size of a burner increases, since the ratio of shell 70 surface to volume decreases as the diameter of the burner is increased. Consequently, as size of the burner is increased (to provide for greater ore capacity), an increased percentage of the total heat generated would normally be carried 75

by the  $\text{SO}_2$  gases leaving the furnace. Since the amount of heat which may be carried out of the burner with the  $\text{SO}_2$  gases is limited (so as to avoid softening of the cinder), in order to provide for disposal by radiation of the greater amount of heat generated it would be necessary to build a burner having about 2.5 times the combustion space of the initial given burner. This obviously involves greatly increased cost of the burner unit. Operation of the plant using a larger new burner is summarized in Example 4 of Table I.

The present invention not only provides elimination of the foregoing difficulties but affords many other substantial operating advantages which will become apparent as the description proceeds.

In the following specific example of practice of the invention, raw materials used are finely divided iron pyrites, for example flotation concentrates, and iron sulfate in the form of the monohydrate  $\text{FeSO}_4 \cdot \text{H}_2\text{O}$ , supplies of which materials are maintained in bins 134 and 138. At start of operations, combustion chamber 17 of furnace 10 is heated by oil burners inserted through workholes not shown to temperatures of 900-1000° F. Pyrites fines alone are then injected and burned until the roaster temperature is raised to about normal, e. g., 1800-1850° F. Subsequently, finely divided pyrites and  $\text{FeSO}_4 \cdot \text{H}_2\text{O}$  are fed into hopper 27 through conduits 135 and 138, proper proportions being maintained by regulation of valves 137 and 138. The raw materials are mixed in conveyor 26 and charged into the top of feed conduit 23. In the preferred embodiment, the air used to supply combustion in the furnace is preheated in heat exchangers 48 and 50. Assuming furnace 10, dust chamber 35 and exchangers 40 and 50 are heated up to normal operating temperatures, air at temperature of about 100° F. is introduced by blower 53 through pipe 54 into the air space in exchanger 50, and heated to temperatures of about 550° F. Such air flows through pipe 58 and is introduced at temperature of about 500° F. into the air space of exchanger 40. The air is discharged through pipe 68 at temperature of about 950° F., and is conducted by pipe 60 to air inlet 30 of furnace feed mechanism 18 which may be of any approved design to effect introduction into combustion chamber 17 of a suspension of finely divided iron pyrites and iron sulfate in air.

On introduction into chamber 17, heated to temperatures above the ignition point of iron sulfide, the pyrites flash to ignition and roasting commences. Suspension roasting of pyrites is highly exothermic and results in formation of a gas mixture comprising  $\text{SO}_2$ , oxygen and nitrogen and in production of iron oxide cinder predominantly  $\text{Fe}_3\text{O}_4$ . In suspension roasting of sulfide fines it is possible to generate much more heat than is necessary to maintain the reaction exothermically self-sustaining.

At temperatures of about 850° F. ferrous sulfate decomposes endothermically to form iron oxide predominantly  $\text{Fe}_2\text{O}_3$  and about equal amounts of  $\text{SO}_2$  and  $\text{SO}_3$ . This reaction proceeds very slowly at this temperature. It has been found that under conditions existing in suspension roasting, with temperatures of the order of 1850° F. prevailing, decomposition of iron sulfate proceeds rapidly and that  $\text{SO}_3$  is dissociated to  $\text{SO}_2$  and oxygen. In customary sulfide fines suspension roasting, it is necessary to limit the amount of fines fed into the combustion chamber so that

the gas temperatures will not exceed the permissible upper limit, e. g. 1900° F. In the process of the present invention, all of the heat in the burner—over and above that lost with the cinder and by radiation, and that required to maintain the roasting operating temperature—is utilized to effect decomposition of iron sulfate. Developments upon which the invention are based show that when iron sulfate fines are introduced along with sulfide fines into a commercial suspension roaster of the type shown in the drawings and having a height such that the fines had a drop of about 25 feet, the iron sulfate is decomposed with the production of an iron oxide cinder containing as little as 0.5% sulfur. While normal endothermic decomposition of iron sulfate at temperatures of about 850° F. results in production of a cinder predominantly  $\text{Fe}_3\text{O}_4$ , on account of the much higher temperatures present in the suspension roasting operation the iron oxide cinder produced by decomposition of the iron sulfate is predominantly  $\text{Fe}_2\text{O}_3$ , i. e., the same form as the iron oxide cinder resulting from suspension roasting of the pyrites fines.

Degree of subdivision of the pyrites may vary over a relatively wide range, preferably not coarser than about 60 mesh. Fineness of the iron sulfate is likewise variable although indications are that better desulfurization of iron sulfate is obtained where the particle size is less than 100 mesh and preferably of the order of 150-200 mesh. In the present specification and claims the term "finely divided" is used to define a degree of subdivision sufficient to permit commercially satisfactory desulfurization of either iron sulfide or iron sulfate. It will be appreciated that height of the burner and the mode of injection of the fines, whether downwardly from the top or upwardly from the bottom or otherwise, influence the time interval during which the fines are maintained in suspension. When using some types of burners the iron sulfide and sulfate should be more finely divided than in the case of others so as to permit lapse of a sufficient time interval in which to complete roasting of the fines while in suspension. The sulfide and sulfate may be charged to the burner by means of separate injectors, although usually better results may be obtained when the fines are introduced in admixture as described.

Reaction conditions in shaft furnace 10 are controlled by regulation of the relative quantities of pyrites fines, iron sulfate fines, and oxygen introduced. The amounts of oxygen and pyrites and sulfate fines charged are regulated so that exothermic combustion of the iron sulfide is effected in such a way as to maintain in the combustion zone temperatures about or above dissociation temperature of sulfur trioxide but preferably not above temperatures which would cause the iron oxide cinder at the point of discharge from the roaster to fuse and set up as a solid cake. By maintaining these conditions, the iron sulfide fines are roasted to produce iron oxide ( $\text{Fe}_3\text{O}_4$ ) cinder and  $\text{SO}_2$  gas; the iron sulfate is decomposed to form iron oxide ( $\text{Fe}_2\text{O}_3$ ) cinder,  $\text{SO}_2$  and  $\text{SO}_3$  gases. The  $\text{SO}_3$  is dissociated to  $\text{SO}_2$  and oxygen; and the sulfur and iron values of the iron sulfide and of the iron sulfate are recovered as a concentrated  $\text{SO}_2$  gas and as relatively free-flowing iron oxide cinder.

The quantities and relative proportions of iron sulfide and sulfate charged to the burner are influenced by several factors such as specific compositions of the sulfide and sulfate, the size and

insulation of the burner, initial temperature of the combustion supporting air, and  $\text{SO}_2$  concentration desired in the burner exit gas.

With respect to the amount of sulfide fines introduced, it will be recalled that in normal sulfide suspension roasting, using pyrites alone, feed of pyrites is limited for a given burner so as to avoid excessive gas temperatures in the combustion chamber. In the present process, no such limitation is encountered. To the contrary, the presence in the combustion zone of as much heat as possible is desirable because the greater the amount of heat available the greater may be the amount of iron sulfate decomposed with resultant increased  $\text{SO}_2$  gas concentration and increased overall capacity of the burner and of the associated sulfuric acid plant. Thus, giving consideration to other factors involved such as size of the furnace, initial temperature of the oxidizing gas, and amount of iron sulfate available for use, the quantity of iron sulfide fed into the burner in the present process is determined according to specific operating conditions existing so as to maintain the reaction as a whole exothermic and to maintain in the combustion zone temperatures, as nearly as practicable, of about 1850° F.

The total air used in the burner in the present process may be considered as the sum of two increments: (1) the amount of air necessary to oxidize the pyrites to  $\text{Fe}_3\text{O}_4$  cinder and gas containing  $\text{SO}_2$ ,  $\text{O}_2$ , and  $\text{N}_2$ ; and (2) an additional amount of air to preferably insure presence in the burner exit gas of the same  $\text{SO}_2$ -oxygen ratio as is present in an  $\text{SO}_2$  gas from pyrites alone. For example, assume the first increment consists of air required to roast the pyrites present and produce a 12%  $\text{SO}_2$  gas. Thus, combustion of pyrites to form a 12%  $\text{SO}_2$  gas results in formation of iron oxide cinder chiefly  $\text{Fe}_3\text{O}_4$  and a gas containing (dry basis) about 12.0%  $\text{SO}_2$ , 5.7%  $\text{O}_2$ , and 82.3%  $\text{N}_2$ , which represents an  $\text{SO}_2$  to oxygen ratio of 1 to 0.47. During roasting of pyrites, decomposition of  $\text{FeSO}_4 \cdot \text{H}_2\text{O}$  simultaneously takes place producing iron oxide chiefly  $\text{Fe}_3\text{O}_4$  and a gas which after condensation of the water vapor would contain about 75%  $\text{SO}_2$  and 25%  $\text{O}_2$ . In this situation, assuming use of air preheated to 900° F., upon mixing the pyrites gas and the iron sulfate gas there would be formed a combined burner exit gas containing (dry basis) 15.9%  $\text{SO}_2$ , 6.9%  $\text{O}_2$ , and 77.2%  $\text{N}_2$ . Since the  $\text{SO}_2$ -oxygen ratio of the burner exit gas in the instance mentioned is 1:0.43 a second increment of air should be introduced into the combustion chamber in amount enough to dilute the combustion gases so that the combined burner exit gas has an  $\text{SO}_2$ -oxygen ratio of about 1:0.47.

The amount of iron sulfate decomposed in a given furnace depends upon the total amount of heat available, and the latter in turn depends upon the amount of iron sulfide burned and upon the temperature of the air as fed into the burner. One of the surprising features of the invention is the unexpected effect of use of preheated air on the capacity or sulfur output of a given furnace. Several prior art suggestions have been made relative to use of preheated air in suspension roasting. Such suggestions are for the most part based on assumption that use of preheated air is beneficial with respect to furnace capacity. However, commercial practice of suspension roasting has shown to the contrary. In Example 1 Table I, using pyrites alone, a given burner and air initially at about 100° F. (atmospheric air 75 in the immediate vicinity of a suspension roaster

is normally about 100° F.) the maximum sulfur output of the burner is 24.6 tons per day (Item 7). Practical experience has shown that in the case of most ores one of the major difficulties in suspension roasting is that too much heat is developed. If more heat units are introduced into the burner in the form of preheated air, since there is already enough required heat present in the combustion zone, it will be seen the only way to avoid excessive gas temperatures is to cut down the sulfide ore input sufficiently to generate a lesser amount of heat equivalent to heat units introduced with the preheated air. For instance, if in Example 1 air were preheated to about 900° F., in order to avoid excessive gas temperatures in the burner it would be necessary to cut down the sulfur input about 65%, that is, from the 25 tons (Item 5) to about 8.6 tons. Hence, in usual suspension roasting of pyrites, preheated air is detrimental and a practical operator knows preheated air necessitates a cut in the ore input tonnage. With this practical knowledge, an operator would expect that preheated air would adversely affect sulfur input tonnage in the present process. To the contrary, however, it has been found that by using preheated air it is not only possible to maintain an initial sulfur input tonnage but to actually largely increase the same.

Example 6 of Table I details operation of a preferred embodiment of the invention and of the results obtained. In the present process, by reason of use of iron sulfate in conjunction with the sulfide fines roasting, it is possible to make use of all of the heat which can be generated by burning sulfide fines. Hence, heat radiation from the burner shell need not be relied upon, as in the prior practice, to provide for dissipation of the excess heat. Accordingly, in the present process it is desirable to insulate the burner shell as well as feasible.

In the present preferred embodiment, the amount of air introduced into the burner is such as to produce at the burner exit a gas containing (dry basis) 15.5%  $\text{SO}_2$ , 7.3%  $\text{O}_2$ , and 77.2%  $\text{N}_2$ . Such gas passes upwardly through supplemental combustion and dust settling chamber 35, Fig. 1 of the drawings, enters the top of exchanger 40 at about 1750° F., leaves thru pipe 46 at about 1275° F., and is discharged from the top of exchanger 50 at about 700-750° F. At this temperature the  $\text{SO}_2$  is relatively non-corrosive and hence a cyclone dust separator 65 made of ordinary sheet steel may be employed. This 15.5%  $\text{SO}_2$  gas (corresponding with the 10%  $\text{SO}_2$  gas Item 10, Example 1) is fed to the head of the wet purification system 67, Item 11, Example 6. Item 12 shows that on account of the largely increased  $\text{SO}_2$  concentration a 35.5% reduction in size of the purification system is made possible. The 15.5%  $\text{SO}_2$  exit gas of wet purification contains insufficient oxygen to facilitate commercial oxidation of  $\text{SO}_2$  in the converter system. Introduction of sufficient air through inlet 133 to provide in the gas stream a ratio of one volume of  $\text{SO}_2$  to 1.1 volumes of free  $\text{O}_2$  reduces the  $\text{SO}_2$  concentration to about 10.6. Summarizing the major results made possible by the invention, using the same burner as in the standard operation, the sulfur output of the burner may be increased from 24.6 tons (Item 7, Example 1) to about 38.1 tons (Item 7, Example 6), the relative capacity or sulfur output of the burner is increased from about 100 to about 155% (Item 8), the purification system may be made 35% smaller, and 75

the drying, converter and absorption units may be made 20% smaller.

In Example 6 the weight of  $\text{FeSO}_4 \cdot \text{H}_2\text{O}$  and iron pyrites charged into the burner was about 1.1 to 1. It will be appreciated the amount of iron sulfate which may be put through the furnace may vary within rather wide limits depending principally upon the composition of the metal sulfide, for example whether iron sulfide or zinc sulfide, upon the degree of preheat of the air fed to the burner, effectiveness of insulation employed, and upon the amount of  $\text{FeSO}_4 \cdot \text{H}_2\text{O}$  available for any specific burner operation.

There may be instances in which a relatively limited quantity of iron sulfate is available and in such case the degree of preheating of the air may be reduced or air preheating dispensed with entirely.

Fig. 2 of the drawings illustrates a plant layout for use in a case where only a limited amount of iron sulfate is available. In this situation, heat is taken out of the system by means of a waste heat boiler 94 instead of being put back into the burner in the form of air preheat as in the system illustrated in Fig. 1. In the present process, the more or less one molecule of water included in the iron sulfate is vaporized in the burner. In instances where a waste heat boiler is employed it is advisable to dry the combustion supporting air to avoid condensation of  $\text{H}_2\text{SO}_4$  in the boiler. In practice of the process as carried out in apparatus of Fig. 2, air is drawn into the system by a blower 80, passed through a standard drying tower 81 and flowed thence through conduit 82 to burner air inlet 30. In furnace 12, roasting of sulfide and decomposition of iron sulfate is generally the same as in burner 10 of Fig. 1.

Example 5 of Table I illustrates an embodiment of the invention which may be carried out in apparatus of Fig. 2 and where air for combustion is not preheated. However, in Example 5 since no heat units are brought into the burner in the form of preheated air there is less heat available for decomposition of iron sulfate and accordingly the tonnage of iron sulfate is reduced from 60 of Example 6 to about 29 (Item 4). In Example 5, about 0.5 lb. of  $\text{FeSO}_4 \cdot \text{H}_2\text{O}$  is fed into the furnace per pound of pyrites fines (Item 6). The gas leaving the burner through outlet 84 (Fig. 2) contains about 13.7%  $\text{SO}_2$  (Item 10), 6.5%  $\text{O}_2$ , and 79.8%  $\text{N}_2$ , and is at temperature of about  $1850^\circ \text{ F}$ . Such gas flows upwardly through supplemental combustion and dust collecting chamber 87, and enters the top of waste heat boiler 84 at about  $1750^\circ \text{ F}$ . The boiler is controlled so that the gas leaving through pipe 104 is at temperatures of about  $650$ – $700^\circ \text{ F}$ .

The basis for the improvements afforded by the invention is utilization of excess heat in the burner to decompose iron sulfate. The more excess heat present the greater may be the proportionate amount of iron sulfate contained in the iron sulfide-iron sulfate furnace charge, with the result that the greater is the proportionate amount of  $\text{H}_2\text{SO}_4$  which may be produced from iron sulfate. In Examples 1 to 6, Table I the iron sulfide was pyrites comprising approximately 46% iron and 50% sulfur. Pyrrhotite, which may be considered as comprising 58% iron and 35% sulfur, is another sulfide ore well adapted for suspension roasting. If the standard burner of Example 1 were changed over to operate on pyrrhotite alone (not using iron sulfate) instead of pyrites alone, on account of the greater iron and lesser sulfur content of pyrrhotite as com-

pared with pyrites, the relative sulfur output of the burner would be substantially decreased, and the plant  $\text{H}_2\text{SO}_4$  production would be cut correspondingly. Hence, an operator is placed at a marked disadvantage if, for any reason, he switches from use of pyrites alone to pyrrhotite alone. However, it has been found, as another surprising feature of the invention, that when roasting iron sulfate in conjunction with pyrrhotite the advantages are still greater than when roasting iron sulfate in conjunction with pyrites. Thus, in the present invention use of pyrrhotite as the sulfide is not a disadvantage (as is the case when substituting pyrrhotite alone for pyrites alone) but is actually a material advantage. This advantage is based on the fact that when, in the present process, pyrrhotite is used a higher proportionate increase in gas concentration is obtained and the proportionate part of the ultimate  $\text{H}_2\text{SO}_4$  product made from iron sulfate is substantially greater than when using iron sulfate and pyrites.

The reason why an operator is placed at a disadvantage with respect to  $\text{H}_2\text{SO}_4$  tonnage production when switching the given standard burner over from burning pyrites alone to burning pyrrhotite alone will be understood from the following.

Example 1 of Table I and Example 7 of Table II respectively show a comparison of operation of an identical burner with pyrites alone and pyrrhotite alone. Burning pyrrhotite alone in conventional hearth roasting results in production of a 7.5–8.0%  $\text{SO}_2$  gas corresponding with the 9.5–10% gas produced when roasting pyrites alone by conventional hearth roasting. Thus in Example 7, it is assumed the representative suspension roaster, burning pyrrhotite alone, is operated so as to produce an 8%  $\text{SO}_2$  gas (Item 10). This 8%  $\text{SO}_2$  pyrrhotite gas (as compared with the 10%  $\text{SO}_2$  pyrites gas Item 10, Example 1) requiring larger purification, contact and absorption systems is the first disadvantage encountered by an operator changing over to pyrrhotite.

Pound per pound pyrrhotite contains a greater amount of iron and lesser amount of sulfur than pyrites. Accordingly, a greater amount of oxygen is used to oxidize the iron of pyrrhotite than in the case of pyrites, and there is a lesser amount of sulfur available for combination with oxygen to form  $\text{SO}_2$  than in the case of pyrites. When operating with pyrrhotite alone, just as in the case of operating with pyrites alone, the exit burner gas should be maintained at, e. g.,  $1850^\circ \text{ F}$ , and this temperature is controlled by the amount of pyrrhotite charged. In burning pyrrhotite to an 8%  $\text{SO}_2$  gas so many heat units go into the gaseous products, because of additional heat units generated in oxidizing the greater iron content and because of the smaller air volume required per pound of pyrrhotite, it would be necessary when switching the standard burner over from pyrites to pyrrhotite to cut the 50 ton ore charge (Item 3, Example 1) to 41.8 tons (Item 3, Example 7). That is, when burning pyrites alone 50 tons of pyrites may be charged, but when burning pyrrhotite alone in the same burner in order to maintain in the burner exit gas the conventional amount of free oxygen and to maintain the say  $1850^\circ \text{ F}$ . temperature in the exit gas, the ore charge to the furnace would be reduced from 50 tons pyrites to 41.8 tons of pyrrhotite. Thus, when burning pyrrhotite alone the furnace ore charge itself would be reduced and pyrrhotite contains about 30% less sulfur than pyrites. The

net result is that when burning pyrites alone the sulfur output of the burner is 24.6 tons and the burner capacity or sulfur output is 100% (Items 7 and 8, Example 1), whereas when burning pyrrhotite alone in the same burner the sulfur output is reduced to 14.2 tons and the burner capacity or sulfur output is reduced to 58% (Items 7 and 8, Example 7). Accordingly, when an operator changes over from pyrites alone to pyrrhotite alone, the second disadvantage is that the burner sulfur output (as sulfur or as  $\text{SO}_2$ ) is reduced from 100% to 58% correspondingly cutting the plant  $\text{H}_2\text{SO}_4$  production from 100% to 58%. The disadvantages of changing a burner over from pyrites to pyrrhotite are plainly evident, and the extent of these disadvantages may be more fully recognized when it is appreciated that in some localities pyrrhotite is the only sulfide ore available.

In Table II the burners of Examples 7-10 are identical with the burners of Examples 1, 2, 5 and 6 of Table I. However, in Table II since the initial burner gas is 8%  $\text{SO}_2$ , the purification system of Example 7 is designed to handle an 8% pyrrhotite gas. Such gas contains about 8%  $\text{O}_2$ , and more oxygen should be introduced into the gas stream just ahead of the drying system to provide the 1:1.1  $\text{SO}_2$  to oxygen ratio. After introduction of air to provide the requisite oxygen, the  $\text{SO}_2$  concentration of the gas entering the drying system would be reduced to about 7.5% (Item 15, Example 7).

Example 7 thus typifies what may be considered a standard operation using the given standard burner and operating on a maximum capacity for such burner on pyrrhotite ore. When roasting pyrrhotite alone, it would be to the operator's advantage to produce a stronger  $\text{SO}_2$  gas so as to make possible use of a smaller purification system as in the case of pyrites. Assume it is desired to produce a 10%  $\text{SO}_2$  pyrrhotite gas (the maximum  $\text{SO}_2$  concentration obtainable by suspension roasting of pyrrhotite alone) to permit use of a 20% smaller purification system. Example 8 of Table II illustrates such operating conditions and shows the burner capacity or sulfur output is reduced from 58% to 37% (Item 8).

If the operator desires to run the burner on pyrrhotite to produce a 10%  $\text{SO}_2$  burner exit gas and obtain the benefit of the 20% size reduction of the purification system and still maintain the same  $\text{H}_2\text{SO}_4$  plant production as in Example 7 he has two alternatives available: first, to use the given standard burner plus a second burner about 55% as large as the given standard; or second, to use a single new burner about twice the size of the given standard. In other words, the alternatives available when burning pyrrhotite are the same as those possible when burning pyrites as illustrated in Examples 3 and 4 of Table I. The objections to the alternatives in the case of roasting pyrrhotite alone are the same as those when roasting pyrites alone.

While combustion of 1 lb. of pyrites generates a slightly greater number of B. t. u.'s than does the combustion of 1 lb. of pyrrhotite, oxidation of 1 lb. of pyrrhotite to  $\text{Fe}_3\text{O}_4$  and  $\text{SO}_2$  requires a smaller weight or volume of air than does oxidation of 1 lb. of pyrites to  $\text{Fe}_3\text{O}_4$  and  $\text{SO}_2$ . The result of this is that in the roasting of pyrrhotite because of the additional B. t. u.'s generated by oxidizing the substantially greater iron content and because of the smaller air volume required per pound of ore, there is produced in the roasting of pyrrhotite a greater number of B. t. u.'s per pound of gaseous

reaction products than when roasting pyrites. Accordingly, although while roasting pyrrhotite alone possesses substantial overall plant capacity disadvantages as compared with pyrites roasted alone, in the roasting of pyrrhotite alone there is more excess heat available for raising the temperature of the reaction zone than in the case of roasting pyrites alone. Accordingly, when roasting pyrrhotite, there is more heat available for decomposing iron sulfate with the result that on applying the principles of this invention to roasting of pyrrhotite, a greater proportion of iron sulfate may be decomposed and a greater proportionate amount of ultimate  $\text{H}_2\text{SO}_4$  product may be made from iron sulfate than when using pyrites as the sulfide ore. While in prior practice it was a disadvantage to roast pyrrhotite alone, the present invention substantially eliminates the gas concentration disadvantage and creates an advantage with respect to the amount of ultimate  $\text{H}_2\text{SO}_4$  product made from iron sulfate.

In the present modification using pyrrhotite as the sulfide ore, maximum economies may be obtained where the air is preheated. Example 10 illustrates an embodiment of the invention using pyrrhotite, air preheated to about 900° F. and the plant layout of Fig. 1 of the drawings.

The burner exit gas, containing (dry basis) about 15%  $\text{SO}_2$ , (Item 10, Example 10), 7.3%  $\text{O}_2$ , and 77.7%  $\text{N}_2$ , and heated to temperatures of about 1850° F., passes through chamber 35, enters the top of heat exchanger 40 at about 1750° F., is introduced through pipe 46 into the bottom of exchanger 50 at temperature of about 1275° F., and is discharged from the top of exchanger 50 through pipe 63 into dust collector 65 at temperature of about 700-750° F.

Example 9 illustrates an embodiment of the invention using pyrrhotite and the plant layout of Fig. 2 of the drawings. Atmospheric air is drawn into the system by blower 80, dried in tower 81, and introduced into furnace air inlet 30 at temperature of about 100° F.

The burner exit gas containing (dry basis) about 13.2%  $\text{SO}_2$  (Item 10, Example 9), 6.5%  $\text{O}_2$ , 80.3%  $\text{N}_2$ , and heated to temperatures of about 1850° F., passes through chamber 87 and at about 1750° F. enters the top of waste heat boiler 94 controlled so that the gas stream is discharged into conduit 104 at temperature of about 700-750° F. and fed into cyclone dust separator 73.

In Examples 5 and 9, using a well insulated burner and unpreheated air, iron sulfate and sulfide fines were used in proportions of about half pound of sulfate to one pound of ore. Where smaller amounts, say half as much iron sulfate is available, the process may be employed to similar advantage. However, as the relative proportion of sulfide is increased, the amount of heat generated is correspondingly increased, and in this situation it is only necessary to less effectively insulate the burner sufficiently to dissipate by radiation the excess heat.

The invention makes possible economic utilization of a low-grade sulfide known on the market as "coal brasses". The term is applied to iron pyrites occurring as seams in coal deposits, and as separated from the coal consists of an impure iron pyrites containing variable percentages of coal which by concentration methods may be reduced in some cases to about 5% carbon content. Brasses of this type thus contain about 42-48% sulfur. This material is relatively unsuited as a substitute for pyrites in prior hearth roasting since the contained carbon would consume so

much oxygen in the roasting operation and form so much Co, that the SO<sub>2</sub> concentration of the resultant roaster gas would be low and comparable with that obtained from pyrrhotite. While the SO<sub>2</sub> concentration of suspension burner exit gases when using pyrites or pyrrhotite alone is normally higher than when roasting pyrites or pyrrhotite alone in a hearth roaster the same objections relative to the use of coal brasses in hearth roasters applies to suspension roasters, namely, dilution of the SO<sub>2</sub> gas by CO<sub>2</sub>. Consequently, although coal brasses run very high in sulfur this material is of little value as compared with straight pyrites and is accordingly available on the market at much lower prices.

When carrying out the present process using coal brasses as a substitute for straight pyrites or pyrrhotite, roasting of the pyrites content of the brasses maintains the exothermic nature of the reaction and also generates excess heat which is utilized to decompose iron sulfate. Although combustion of the carbon content of the brasses to CO<sub>2</sub> generates substantial amounts of heat, such heat units are not needed to maintain the exothermic nature of the reaction but are available to decompose still further quantities of iron sulfate. Decomposition of iron sulfate produces a very strong SO<sub>2</sub> gas which after condensation of water vapor would contain about 75% SO<sub>2</sub> and 25% oxygen. Such SO<sub>2</sub> gas before introduction into the converters, must in any event be substantially diluted either by air introduced into the burner or fed into the gas stream just ahead of the drying unit or both. Consequently, in present modification of the invention using coal brasses the diluting effects of the CO<sub>2</sub> formed by combustion of the carbon content of the brasses are unobjectionable. For example, FeSO<sub>4</sub>.H<sub>2</sub>O and coal brasses (assumed to contain about 5% carbon by weight) may be introduced into the combustion chamber in proportion of about 0.78 lb. of FeSO<sub>4</sub>.H<sub>2</sub>O to 1 lb. of coal brasses. When using air initially at atmospheric temperature and operating to maintain the burner exit gas temperature at about 1850° F., the resulting burner gas may contain (dry basis) 12.7% SO<sub>2</sub>, 6.0% O<sub>2</sub>, 78.1% N<sub>2</sub> and 3.2% CO<sub>2</sub>. It is thus possible, in spite of CO<sub>2</sub> dilution, to produce a concentrated burner gas. In this instance, the H<sub>2</sub>SO<sub>4</sub> production from the brasses amounts to about 74% of the total, and the H<sub>2</sub>SO<sub>4</sub> production from FeSO<sub>4</sub>.H<sub>2</sub>O is about 26% of the total.

Still greater consumption of iron sulfate may be had where the air introduced into the burner is preheated. Assuming air preheat of about 900° F., FeSO<sub>4</sub>.H<sub>2</sub>O and coal brasses may be fed into the combustion chamber in proportions of about 1.37 pounds of FeSO<sub>4</sub>.H<sub>2</sub>O to 1 lb. of brasses. The burner exit gas may contain (dry basis) 14.4% SO<sub>2</sub>, 6.8% O<sub>2</sub>, 75.8% N<sub>2</sub>, and 3.0% CO<sub>2</sub>. The H<sub>2</sub>SO<sub>4</sub> production from brasses may comprise about 62% of the total and the H<sub>2</sub>SO<sub>4</sub> production from FeSO<sub>4</sub>.H<sub>2</sub>O about 38% of the total.

The above description applies to a coal brass concentrate which is produced in relatively small quantities since the cost of equipment and operation affords little economic justification for application of concentration process. However, in some bituminous fields, where soft coal as mined contains from 2% to 4% sulfur, the coal is subjected to a washing operation resulting in production of clean coal and large quantities of a refuse coal which may be as high as 20-22% sulfur. It is this refuse material that is subjected to concentration methods to produce the previously

referred to "brasses" concentrate. The refuse is unsaleable for coal on account of the high sulfur content, and is not usable for manufacture of H<sub>2</sub>SO<sub>4</sub> by the customary roasting methods because of the high carbon content. However, such refuse may be employed in the present process since the heat developed by combustion of the higher carbon content may be used to decompose further amounts of iron sulfate, the strong SO<sub>2</sub> produced from iron sulfate offsetting CO<sub>2</sub> dilution. 10

The invention thus affords two very distinct additional advantages: first, in that it makes possible economic utilization of a very low-priced raw material, i. e., coal brasses or coal refuse; and further, that when employing such materials the 15 proportionate part of the total H<sub>2</sub>SO<sub>4</sub> production from iron sulfate is greater than when using iron sulfate in conjunction with either pyrites or pyrrhotite ore. Another outstanding advantage of the process of the invention is that when using, 20 in conjunction with the sulfate, either pyrites, pyrrhotite or pyrites containing coal it is possible to produce an SO<sub>2</sub> gas as strong as can be made by burning brimstone, the highest grade 25 of sulfur raw material.

The principles of the invention as described in connection with use of iron sulfide and iron sulfate apply equally to use of zinc sulfide ores and zinc sulfate. It is preferred to use the sulfide and sulfate of the same metal so that the burner 30 cinder will consist of the oxide of a single metal. However, where the situation is such that cinder comprising the oxide of more than one metal is unobjectionable, the sulfide in the present process may be the sulfide of one metal, and the sulfate 35 and sulfate of another metal. The higher oxide of the sulfate, such as ferric sulfate may also be used in place of the lower oxide such as ferrous sulfate. Elemental sulfur may be substituted for sulfate ore, although for practical purposes there 40 would be little or no reason in using a relatively expensive, high-priced raw material in place of the cheaper sulfide.

The iron sulfate mentioned in the foregoing examples contains approximately one molecule of 45 water. For practical purposes the monohydrate is preferred because the water content is relatively low and vaporization of such amount of water in the burner does not consume objectionable amounts of heat. Further, the one water salt is 50 readily obtainable by known crystallizing processes. The anhydrous sulfate may of course be used to even greater advantage than the monohydrate. In the appended claims the expression 55 relatively dehydrated sulfate is intended to include a salt containing about one or less molecules of water. The water content of the iron or other sulfate used in the present process is not critical but is more an operating feasibility. The principles of the invention likewise apply when the 60 salt contains more than one water, e. g., copperas. However, in this situation much heat is needed to vaporize the waters with the result that the quantity of FeSO<sub>4</sub> which may be decomposed would be substantially decreased. If the sulfate 65 is initially available in the seven water form it is more advisable to preliminarily dehydrate down to about one water in a suitable dryer.

While the roasting operation per se has been described as being carried out in the burner of 70 the type disclosed in the Cordy et al. Patent 1,758,188, other types of burners may be employed such for example as shown in Mullen United States Patents 2,070,235 and 2,070,236 of February 9, 1937. 75

TABLE I

Sulfide ore used: Iron pyrites ( $FeS_2$ , 46% Fe, 50% S)

| 5   | Item                                                                                                                                    | Example 1                                                                                                                                                   | Example 2                                              | Example 3                                                             | Example 4                                                        | Example 5                        | Example 6                        | 5     |
|-----|-----------------------------------------------------------------------------------------------------------------------------------------|-------------------------------------------------------------------------------------------------------------------------------------------------------------|--------------------------------------------------------|-----------------------------------------------------------------------|------------------------------------------------------------------|----------------------------------|----------------------------------|-------|
| 1.  | Temp. of air at burner air inlet.                                                                                                       | 100° F.                                                                                                                                                     | 100° F.                                                | 100° F.                                                               | 100° F.                                                          | 100° F.                          | 900° F.                          |       |
| 2.  | Type of burner                                                                                                                          | Given standard.                                                                                                                                             | Given stand-ard.                                       | Given stand-ard plus a second burner 70% as large as given stand-ard. | A single new burner about 2.5 times the size of given stand-ard. | Given stand-ard well in-sulated. | Given stand-ard well insu-lated. | 10    |
| 10  |                                                                                                                                         |                                                                                                                                                             |                                                        |                                                                       |                                                                  |                                  |                                  |       |
| 3.  | Ore charge, net tons per day.                                                                                                           | 50.0                                                                                                                                                        | 29.2                                                   | 50.0 (total of both burn-ers).                                        | 50.0                                                             | 56.0                             | 55.0                             |       |
| 15  | 4.                                                                                                                                      | Fe <sub>2</sub> O <sub>3</sub> .H <sub>2</sub> O charge, net tons per day.                                                                                  | 0                                                      | 0                                                                     | 0                                                                | 0                                | 29.0                             | 60.5  |
| 5.  | Sulfur to burner, net tons per day.                                                                                                     | 25.0                                                                                                                                                        | 14.6                                                   | 25.0 (total of both burn-ers).                                        | 25.0                                                             | 33.0                             | 38.0                             |       |
| 20  | 6.                                                                                                                                      | Pounds of Fe <sub>2</sub> O <sub>3</sub> .H <sub>2</sub> O per pound of sulfide ore.                                                                        | 0                                                      | 0                                                                     | 0                                                                | 0                                | 0.5                              | 1.1   |
| 7.  | Sulfur ex burner, net tons per day.                                                                                                     | 24.6                                                                                                                                                        | 14.3                                                   | 24.6 (total of both burn-ers).                                        | 24.6                                                             | 32.3                             | 38.1                             | 20    |
| 8.  | Relative burner capacity (sulfur output).                                                                                               | 100%                                                                                                                                                        | 58%                                                    | 100% (total of both burn-ers).                                        | 100%                                                             | 131%                             | 155%                             |       |
| 25  | 9.                                                                                                                                      | Temp. of SO <sub>2</sub> gas at burner exit.                                                                                                                | 1,850° F.                                              | 1,850° F.                                                             | 1,850° F.                                                        | 1,850° F.                        | 1,850° F.                        | 25    |
| 10. | SO <sub>2</sub> concentration at burner exit.                                                                                           | 10%                                                                                                                                                         | 12%                                                    | 12%                                                                   | 12%                                                              | 13.7%                            | 15.5%                            |       |
| 11. | SO <sub>2</sub> concentration in wet purification plant (coolers, scrubbers, etc.).                                                     | 10%                                                                                                                                                         | 12%                                                    | 12%                                                                   | 12%                                                              | 13.7%                            | 15.5%                            |       |
| 30  | 12.                                                                                                                                     | Percent reduction in size of purification system.                                                                                                           | None (given size for 10% SO <sub>2</sub> pyrites gas). | 16.7%                                                                 | 16.7%                                                            | 16.7%                            | 27.0%                            | 35.5% |
| 13. | Percent of additional H <sub>2</sub> SO <sub>4</sub> producible in given purification plant by increased SO <sub>2</sub> concentration. | None                                                                                                                                                        | 20%                                                    | 20%                                                                   | 20%                                                              | 37%                              | 55%                              |       |
| 35  | 14.                                                                                                                                     | Air introduced at head of drying unit.                                                                                                                      | Yes                                                    | Yes                                                                   | Yes                                                              | Yes                              | Yes                              | Yes   |
| 15. | SO <sub>2</sub> concentration in drying, converter and absorption units.                                                                | 8.5%                                                                                                                                                        | 8.5%                                                   | 8.5%                                                                  | 8.5%                                                             | 9.7%                             | 10.6%                            | 35    |
| 16. | Percent reduction in size of drying, converter and absorption units.                                                                    | None (given size for 8.5% SO <sub>2</sub> pyrites gas).                                                                                                     | None                                                   | None                                                                  | None                                                             | 12.0%                            | 20.0%                            |       |
| 40  | 17.                                                                                                                                     | Percent of additional H <sub>2</sub> SO <sub>4</sub> producible in given drying, converter and absorption units by increased SO <sub>2</sub> concentration. | None                                                   | None                                                                  | None                                                             | None                             | 14%                              | 25%   |
| 18. | H <sub>2</sub> SO <sub>4</sub> production from ore.                                                                                     | 100%                                                                                                                                                        | 100%                                                   | 100%                                                                  | 100%                                                             | 83.4%                            | 70.5%                            |       |
| 45  | 19.                                                                                                                                     | H <sub>2</sub> SO <sub>4</sub> production from Fe <sub>2</sub> O <sub>3</sub> .H <sub>2</sub> O.                                                            | 0                                                      | 0                                                                     | 0                                                                | 16.6%                            | 29.5%                            | 45    |

TABLE II

Sulfide ore used: Pyrrhotite ( $Fe_7S_8$ , 58% Fe, 35% S)

| 50  | Item                                                                                                                                                          | Example 7                                                                            | Example 8                                                  | Example 9                        | Example 10                       | 50                               |    |
|-----|---------------------------------------------------------------------------------------------------------------------------------------------------------------|--------------------------------------------------------------------------------------|------------------------------------------------------------|----------------------------------|----------------------------------|----------------------------------|----|
| 55  | 1.                                                                                                                                                            | Temp. of air at burner air inlet.                                                    | 100° F.                                                    | 100° F.                          | 100° F.                          | 900° F.                          | 55 |
| 2.  | Type of burner                                                                                                                                                | Given standard (iden-tical with "standard" of Table I).                              | Given stand-ard.                                           | Given stand-ard well in-sulated. | Given stand-ard well insu-lated. | Given stand-ard well insu-lated. |    |
| 3.  | Ore charge, net tons per day.                                                                                                                                 | 41.8                                                                                 | 27.0                                                       | 67.0                             | 67.0                             |                                  |    |
| 4.  | Fe <sub>2</sub> O <sub>3</sub> .H <sub>2</sub> O charge, net tons per day.                                                                                    | 0                                                                                    | 0                                                          | 41.5                             | 73.7                             |                                  |    |
| 5.  | Sulfur to burner, net tons per day.                                                                                                                           | 14.6                                                                                 | 9.5                                                        | 31.3                             | 37.3                             |                                  |    |
| 60  | 6.                                                                                                                                                            | Pounds of Fe <sub>2</sub> O <sub>3</sub> .H <sub>2</sub> O per pound of sulfide ore. | 0                                                          | 0                                | 0.6                              | 1.1                              | 60 |
| 7.  | Sulfur ex burner, net tons per day.                                                                                                                           | 14.2                                                                                 | 9.2                                                        | 30.3                             | 38.2                             |                                  |    |
| 8.  | Relative burner capacity (sulfur output).                                                                                                                     | 55%                                                                                  | 37%                                                        | 123%                             | 147%                             |                                  |    |
| 9.  | Temp. of SO <sub>2</sub> gas at burner exit.                                                                                                                  | 1,850° F.                                                                            | 1,850° F.                                                  | 1,850° F.                        | 1,850° F.                        |                                  |    |
| 10. | SO <sub>2</sub> concentration at burner exit.                                                                                                                 | 8%                                                                                   | 10%                                                        | 13.2%                            | 15.0%                            |                                  |    |
| 11. | SO <sub>2</sub> concentration in wet purification plant (coolers, scrubbers, etc.).                                                                           | 8%                                                                                   | 10%                                                        | 13.2%                            | 15.0%                            |                                  |    |
| 65  | 12.                                                                                                                                                           | Percent reduction in size of purification system.                                    | None (given size for 8% SO <sub>2</sub> pyrrhotite gas).   | 20.0%                            | 39.4%                            | 46.7%                            | 65 |
| 13. | Percent of additional H <sub>2</sub> SO <sub>4</sub> producible in given puri-fication plant by increased SO <sub>2</sub> concentration.                      | None                                                                                 | 25%                                                        | 65%                              | 87.5%                            |                                  |    |
| 14. | Air introduced at head of drying unit.                                                                                                                        | Yes                                                                                  | Yes                                                        | Yes                              | Yes                              |                                  |    |
| 15. | SO <sub>2</sub> concentration in drying, converter and absorption units.                                                                                      | 7.5%                                                                                 | 7.5%                                                       | 9.5%                             | 10.4%                            |                                  |    |
| 70  | 16.                                                                                                                                                           | Percent reduction in size of drying, converter and absorption units.                 | None (given size for 7.5% SO <sub>2</sub> pyrrhotite gas). | None                             | 21.0%                            | 28.0%                            | 70 |
| 17. | Percent of additional H <sub>2</sub> SO <sub>4</sub> producible in given dry-ing, converter, and absorption units by increased SO <sub>2</sub> concentration. | None                                                                                 | None                                                       | 27%                              | 39%                              |                                  |    |
| 18. | H <sub>2</sub> SO <sub>4</sub> production from ore.                                                                                                           | 100%                                                                                 | 100%                                                       | 75.1%                            | 62.6%                            |                                  |    |
| 19. | H <sub>2</sub> SO <sub>4</sub> production from Fe <sub>2</sub> O <sub>3</sub> .H <sub>2</sub> O.                                                              | 0                                                                                    | 0                                                          | 24.0%                            | 37.4%                            |                                  |    |

I claim:

1. The method for roasting metal sulfide fines which comprises introducing metal sulfide fines, metal sulfate fines and oxidizing gas into a combustion zone heated to temperatures above the ignition point of the sulfide fines, forming in the combustion zone a dispersion of the sulfide and sulfate fines in the oxidizing gas, roasting the sulfide fines while in gaseous suspension, regulating the amount of sulfate introduced so as to avoid reducing combustion zone temperature below that at which sulfide fines introduced into the combustion zone ignite and oxidize in the presence of oxygen, causing the sulfide and sulfate fines to pass through the combustion zone so as to maintain such fines in suspension for a sufficient time interval to roast the sulfide fines and to decompose the sulfate fines to form from the sulfide and sulfate fines sulfur dioxide gas and substantially desulfurized metal oxide cinder, withdrawing sulfur dioxide from the combustion zone, and discharging cinder therefrom.
2. The method for roasting metal sulfide fines which comprises introducing metal sulfide fines, metal sulfate fines and oxidizing gas into a combustion zone heated to temperatures above the ignition point of the sulfide fines, forming in the combustion zone a dispersion of the sulfide and sulfate fines in the oxidizing gas, roasting the sulfide fines while in gaseous suspension, regulating the amount of sulfate introduced so as to avoid reducing combustion zone temperature below that effecting substantial dissociation of sulfur trioxide, causing the sulfide and sulfate fines to pass through the combustion zone so as to maintain such fines in suspension for a sufficient time interval to roast the sulfide fines and to decompose the sulfate fines to form from the sulfide and sulfate fines sulfur dioxide gas and substantially desulfurized metal oxide cinder, withdrawing sulfur dioxide from the combustion zone, and discharging cinder therefrom.
3. The method according to claim 1 in which the amount of sulfate introduced is regulated so as to prevent combustion zone temperature above that causing metal oxide cinder at the point of discharge from the combustion zone to form solid cake.
4. The method according to claim 1 in which the oxidizing gas is preheated.
5. The method according to claim 1 in which the fines are sulfide and sulfate of iron.
6. The method for roasting metal sulfide fines which comprises introducing oxidizing gas, metal sulfide fines and relatively dehydrated metal sulfate fines in proportion of about one to not less than about 0.5 by weight into a combustion zone heated to temperatures above the ignition point of the sulfide fines, forming in the combustion zone a dispersion of the sulfide and sulfate fines in the oxidizing gas, roasting the sulfide fines while in gaseous suspension, causing the sulfide and sulfate fines to pass through the combustion zone so as to maintain such fines in suspension for a sufficient time interval to roast the sulfide fines and to decompose the sulfate fines to form

from the sulfide and sulfate fines sulfur dioxide gas and substantially desulfurized metal oxide cinder, withdrawing sulfur dioxide from the combustion zone, and discharging cinder therefrom.

7. The method according to claim 6 in which the amount of sulfate introduced is regulated so as to prevent combustion zone temperature above that causing metal oxide cinder at the point of discharge from the combustion zone to form solid cake.

8. The method according to claim 6 in which the oxidizing gas is preheated at least several hundred degrees F., and the sulfide fines and sulfate fines are in proportion of about one to not less than about one by weight.

9. The method for roasting finely divided combustible solid sulfur bearing material which comprises introducing said material, metal sulfate fines and oxidizing gas into a combustion zone heated to temperatures above the ignition point of the sulfur bearing material, forming in the combustion zone a dispersion of the sulfur bearing material and sulfate fines in the oxidizing gas, roasting the said material while in gaseous suspension, regulating the amount of sulfate introduced so as to avoid reducing combustion zone temperature below that at which the sulfur bearing material introduced into the combustion zone ignites and oxidizes in the presence of oxygen, causing the sulfur bearing material and sulfate fines to pass through the combustion zone while in suspension for a sufficient time interval to oxidize the sulfur of said material and to decompose the sulfate fines to form sulfur dioxide gas and substantially desulfurized metal oxide cinder, withdrawing sulfur dioxide from the combustion zone, and discharging cinder therefrom.

10. The method according to claim 1 in which the fines are sulfide and sulfate of the same metal.

11. The method according to claim 1 in which the sulfate fines are relatively dehydrated.

12. The method according to claim 2 in which the amount of sulfate introduced is regulated so as to prevent combustion zone temperature above that causing metal oxide cinder at the point of discharge from the combustion zone to form solid cake.

13. The method according to claim 2 in which the fines are sulfide and sulfate of iron.

14. The method according to claim 2 in which the metal sulfate fines are relatively dehydrated, and metal sulfide fines and relatively dehydrated metal sulfate fines are introduced into the combustion zone in proportion of about one to not less than 0.5 by weight.

15. The method according to claim 6 in which the fines are sulfide and sulfate of the same metal.

16. The method according to claim 9 in which the finely divided combustible solid sulfur bearing material is coal brasses.

17. The method according to claim 9 in which the sulfate fines are relatively dehydrated.